

## UNITED STATES PATENT OFFICE

THEODORE F. BRADLEY, OF WESTFIELD, NEW JERSEY, ASSIGNOR TO ELLIS-FOSTER COMPANY, OF MONTCLAIR, NEW JERSEY, A CORPORATION OF NEW JERSEY

## FINGER NAIL GLOSSIFIER

No Drawing.

Application filed July 16, 1928. Serial No. 293,319.

This invention relates to a perfume-responsive finger-nail glossifier composed of solid gloss-producing substances including nitrocellulose of special characteristics, dissolved in a highly-volatile perfume-responsive solvent comprising ethyl alcohol and other solvents present in minor proportions.

The object of the invention is to produce a glossifier having the following qualities:

10 1. Quick-drying; so that when applied as a coating of sufficient thickness to secure a good gloss, drying will not require more than one minute.

15 2. Perfume-responsive; that is, possessing so slight or mild an odor it is possible to introduce very small proportions of costly perfume oils such as oil of rose to give the composition a flowery odor or bouquet. Thus there are excluded in any substantial proportion

20 from the glossifier vehicle all that class of nitrocellulose solvents comprised by the well-known term "banana liquid".

25 3. Clarity and color; the initial untinted glossifier being free from turbidity and coloration, lending itself readily to tinting with red or pink dyes.

30 4. Freedom from discoloration; since on standing, especially when exposed to light nitrocellulose of low viscosity (referred to below) is not wholly stable and may alter slightly with consequent action on some perfume oils to create discoloration. Perfume oils, when used, should be color-stable under these conditions.

35 5. High gloss; a term meaning that one or two applications of the glossifier will form a coating of the requisite gloss.

40 6. Adhesion; the coating should possess good adhesion over a reasonable period, must not crack, peel, nor be harmed by prolonged contact with soapy water and various other ordinary household fluids with which the hands often come in contact.

45 7. Color-stability of aged coatings; the thin film of glossifier on the finger-nails should not turn yellow or show any other perceptible discoloration within the contemplated period of exposure and wear.

8. Dye-stability; when dyes are used to give a shell-pink color or similar tone or tint

to the dried coating, the dye should be stable in color value and should not wash out. In a layer so thin as the gloss coating secured by the use of the present glossifier, employing low-viscosity nitrocellulose with its lowered stability (compared with high viscosity nitrocellulose) dyes which are objectionably acted on in the course of time in the dried film due to changes taking place in the nitrocellulose, should be avoided.

9. Smoothness of coating; "banana liquid" is often used as a slow-drying solvent to smooth out the coating, prevent "orange peel" and overcome blushing. One minute drying means the employment of much more volatile solvents with consequent difficulty in securing a perfect film. The solvent vehicle of the present invention is adapted to yield smoothness and transparency in wholly adequate degree.

In order to obtain a glossifier medium which possesses the highly important property of quick-drying, I find it necessary to use substantially only highly volatile solvents and to use as the solid gloss-producing material practically only nitrocellulose, preferably of low viscosity, without material additions of resins, drying oils and various other substances such as are usually put into various nitrocellulose coating compositions. The solvents available also are restricted in number because I aim to use only solvents having practically no odor, or, at most, possessing a mildly odorous nature, capable of being masked by the employment of a modicum of a perfuming agent. A further limitation with respect to the solvent is that preferably it should be of a pale or water-white transparent nature and possessing a light-stable quality. This eliminates certain solvents such as mesityl oxide, and the like, which darken badly on exposure to sunlight. Furthermore, the solvents employed should not contain objectionable impurities or substances which will affect the color or the gloss-producing solids used in the glossifier composition.

These requirements therefore preclude the use of a great number of solvents employed in industrial nitrocellulose solutions, espe-

cially such solvents as butyl and amyl alcohols and their esters which compose the bulk of the so-called "banana oil". The use of many other heavier solvents is likewise precluded because of their slow rate of evaporation. Thus, there are certain solvents obtained from glycol such as the mono ethyl ether of ethylene glycol which, while not possessing an odor, are so slow in drying that they do not provide a glossifier meeting my very restricted specifications.

Furthermore, the employment of any substantial proportion of ketones of low boiling point, such as acetone and methyl ethyl ketone, is objectionable because these solvents are not sufficiently perfume-responsive due to their penetrating odors. The esters of the lower alcohols such as methyl acetate, ethyl acetate, isopropyl acetate, and the like, also are not adequately perfume-responsive. Relatively small proportions of some of these which yield good solvents for nitrocellulose, but are lacking in perfume-responsiveness, may, however, be used, provided the content of these highly volatile moderately odorous solvents does not exceed the perfume-responsiveness limit. The most satisfactory vehicle for the nitrocellulose, I find to be anhydrous ethyl alcohol. It is, however, a poor solvent for nitrocellulose, especially for those grades of low-viscosity nitrocellulose which are stable to light. There are certain nitrocelluloses which are more soluble in ethyl alcohol, but these I have observed are more readily discolored by light. Hence, a solution made with such light-stable nitrocellulose on standing on the shelves exposed to light for some time is likely to change color and be rejected by the prospective user.

In order to fortify the anhydrous ethyl alcohol to make it more generally applicable for the employment of light-stable nitrocellulose of low viscosity, I use a strengthening solvent fortifier such as anhydrous methyl alcohol or methanol and preferably employ it only to the extent of from 10 to 20 per cent of the total volume of the total solvent vehicle. Thus, I may use from 80 to 90 parts by volume of anhydrous ethyl alcohol and 10 to 20 parts of anhydrous methyl alcohol. Using this as a fortifier in the low proportions stated, I am able to make a nitrocellulose solution containing a sufficiently high content of nitrocellulose solids that I can secure a good coating and high gloss with only one application to the finger nails.

In addition to ethyl alcohol, I may sometimes employ isopropyl and tertiary butyl alcohols, either alone or in admixture with ethyl alcohol as the major alcoholic basis and employ with these a proportion of methanol or other fortifier adequate to convey the requisite solvent properties on nitrocellulose. The anhydrous ethyl alcohol is, however, milder in odor than either the isopropyl or

the tertiary butyl alcohol and therefore in the preferred form of the invention ethyl alcohol constitutes the major part of the solvent vehicle.

Other fortifiers may include small percentages of acetone, methyl ethyl ketone, methyl and ethyl acetates, and the like, bearing in mind that these are preferably kept within limits of perfume-responsiveness. Low viscosity nitrocellulose solutions are frequently improved in quality by the addition of benzol, toluol, or even in some cases, low boiling point petroleum hydrocarbons. The employment of hydrocarbons, especially of the aromatic series, sometimes enables a better solution of the nitrocellulose and the deposition of smoother and more glossy films, especially when used in conjunction with ethyl alcohol and a fortifier, as aforesaid.

A solvent vehicle suitable for the purpose is made from the following approximate proportions by volume.

|                           | Parts |
|---------------------------|-------|
| Anhydrous ethyl alcohol   | 80    |
| Anhydrous methyl alcohol  | 15    |
| Toluol                    | 5     |
| Light gasoline distillate | 4     |
| Ethyl acetate             | 6     |

Using 80 to 90 parts by weight of this solvent vehicle, I dissolve therein from 10 to 15 parts of nitrocellulose of a viscosity preferably one-half second or lower.

Compositions made according to the foregoing being free from resins and substances retarding evaporation, will be found to dry in less than one minute when applied by means of a small brush to the finger nails in a layer of customary coating thickness. On drying, clear transparent films possessing high gloss and adequate adhesion result. During the entire drying period the odor is so mild as to be negligible and there is no retention of slow drying substances having an objectionable odor, such as result from the customary use in the lacquer industry of various high-boiling solvents.

As previously stated, perfumes employed in the foregoing perfume-responsive vehicle should be light-stable. I have found that various essential oils offered as perfumes turn yellow or brown in solution on exposure to light and in the nitro-cellulose films on the nails. In other cases, perfuming oils are incompatible with nitrocellulose and may even cause precipitation of the latter or the formation of a blushed coating. It is important that the coating on the nails be thoroughly transparent, hence any substance which causes blushing should be avoided. I have found that several of the rose perfumes such as oil of rose in well refined form are sufficiently light-stable to be used in a glossifier of the type illustrated herein. In view of the perfume-responsive character of the vehicle the proportion of oil of rose required is small,

but can, of course, be varied in accordance with individual requirements. In any event, only a modicum of the oil of rose is required, as for example, 10 to 20 drops of the oil in 12 to 16 fluid ounces of the glossifier.

The dye or coloring matter previously referred to preferably should be present in proportion sufficient to give a flesh-pink or shell-pink color or a stronger pinkish or reddish 10 coloration, as desired. Other tones or tints may be employed, as desired, but pink or rose colors are generally preferable. Only such dyes should be used as are unaffected by water and other compounds with which the 15 hands may come in contact. The dye also should be as chemically inert as possible and should be compatible with the other ingredients of the glossifier.

Thus, there is obtained a finger nail glossifier comprising nitrocellulose of approximately not over one-half second viscosity, a modicum of a perfume oil color-stable in the presence of low viscosity nitrocellulose and a substantially color-stable dye, producing 20 a shell-pink or rose-pink tint in the dried coating, all dissolved in a perfume-responsive solvent vehicle substantially free from "banana oil" and comprising ethyl alcohol as the major solvent and a mixture of other volatile solvents within the perfume-responsive 25 range as the minor solvent; said glossifier when applied to the finger nails as a layer of gloss-producing thickness drying in a period of less than one minute to a smooth 30 glossy transparent coating free from "orange peel" defacement.

Many volatile solvent mixtures produce a rippling of the surface which is known as "orange peel" and the absence of this effect 40 in the composition aforesaid makes the composition particularly desirable as a finger nail glossifier.

It should be noted that the employment of nitrocellulose of high viscosity under such 45 circumstances does not yield a sufficient content of solid material to enable high gloss to be developed. Moreover, the very thick heavy-bodied compositions resulting from the high viscosity nitrocellulose cannot be applied very smoothly, especially when highly volatile solvent vehicles are used. The composition therefore revolves about the employment of nitrocellulose of low viscosity, usually of a rating less than one second, and 55 preferably of a rating less than one-half second. Solvents which are highly volatile such as methyl and ethyl alcohol and acetone yield solutions of a minimum of viscosity, whereas, the introduction of various high- 60 boiling solvents of a water-eliminating character tend to increase the viscosity. Since, as indicated, a maximum content of solid material is desired in order to create adequate gloss with one application the low viscosity 65 nitrocellulose and the highly volatile solvents

aforesaid cooperate in securing this result. The concentration should not, however, be so high that the flowing and drying qualities are impaired yielding irregular films which are not sufficiently smooth to be practicable. 70 Neither should the concentration be so low that one has to apply several coats to attain the desired glossy finish. I preferably employ a concentration which will give adequate gloss in one application, or at the most, 75 in two such applications.

When the desired high gloss finish is to be obtained with one application, it is advisable to employ at least 12 per cent of nitrocellulose in the solution. Under such circumstances 80 nitrocellulose of one-fourth second viscosity may be used.

One formula employing nitrocellulose of one-fourth second viscosity is the following:

A solvent vehicle was prepared in approximately the following proportions, these being parts by volume:

|                           | Parts |
|---------------------------|-------|
| Anhydrous ethyl alcohol   | 56    |
| Anhydrous methyl alcohol  | 3     |
| Acetone                   | 8     |
| Ethyl acetate             | 4     |
| Light gasoline distillate | 3     |
| Toluol                    | 4     |

To 78 parts by weight of this solvent vehicle I employ 22 parts of the one-fourth second nitrocellulose, adding dye and perfume oil as aforesaid, yielding a good readily-flowable glossifier which provides an excellent gloss finish on the application of one coat to the finger nails.

Likewise, in some cases solvents of higher boiling point may be employed in small proportions, the solvent vehicle being made as follows, expressed in parts by volume.

|                           | Parts |
|---------------------------|-------|
| Anhydrous ethyl alcohol   | 57    |
| Ethyl acetate             | 9     |
| Anhydrous methyl alcohol  | 2     |
| Toluol                    | 4     |
| Light gasoline distillate | 3     |
| Methyl oxybutyrate        | 5     |

20 parts by weight of nitrocellulose of one-fourth second viscosity was dissolved in 80 parts by weight of this solvent vehicle, the nitrocellulose containing 30 per cent of alcohol.

Both the compositions last mentioned are perfume-responsive and capable of carrying dyes, as described.

A glossifier which is free from hydrocarbons may be made in the following manner:

Nitrocellulose of one-fourth second viscosity containing 30 per cent of alcohol is dissolved in a mixture of 85 volumes of anhydrous ethyl alcohol and 15 volumes of acetone. The nitrocellulose content may range from 10 to 19 per cent. Another composition may be made in like manner by using ethyl acetate in lieu of acetone. These solutions dry to a

clear transparent and glossy coating on the finger nail. If 95 per cent ethyl alcohol is used, opaque or milky coatings result.

Still another glossifier was made from the 8 one-fourth second viscosity nitrocellulose dissolved in a mixture of 80 volumes of 98 per cent isopropyl alcohol and 20 volumes of ethyl acetate. Replacement with acetone of one-half of the ethyl acetate used in the last 10 mentioned formula caused severe blushing.

11 What I claim is:—

12 1. A finger-nail glossifier comprising 15 nitrocellulose of approximately not over one half-second viscosity, a modicum of a perfume oil color-stable in the presence of low viscosity nitrocellulose and a substantially color-stable dye producing a shell-pink tint in the dried coating, all dissolved in a perfume-responsive solvent vehicle substantially 20 free from "banana oil" and comprising ethyl alcohol as the major solvent and a mixture of other volatile solvents within the perfume-responsive range as the minor solvent; said glossifier when applied to the finger nails 25 as a layer of gloss-producing thickness drying in a period of less than one minute to a smooth glossy transparent coating free from "orange peel" defacement.

26 2. A finger nail glossifier comprising 30 nitrocellulose of approximately not over one half second viscosity, a modicum of a perfume oil color-stable in the presence of low viscosity nitrocellulose, dissolved in a perfume-responsive solvent vehicle substantially 35 free from "banana oil" and comprising ethyl alcohol as the major solvent and a mixture of other volatile solvents within the perfume-responsive range as the minor solvent; said glossifier when applied to the finger nails as 40 a layer of gloss-producing thickness drying in a period of less than one minute to a smooth glossy transparent coating free from "orange peel" defacement.

45 3. A finger nail glossifier composition consisting of low viscosity nitrocellulose dissolved in substantially anhydrous ethyl alcohol and synthetic methanol in proportions to yield a substantially blush-free coating on drying.

50 4. A finger nail glossifier composition comprising low viscosity nitrocellulose and a composite solvent including ethyl alcohol and methyl alcohol, the proportions of these alcohols in the solvent being from 80 to 90 parts 55 by volume of ethyl alcohol to 20 to 10 parts of methyl alcohol.

56 5. A finger nail glossifier composition comprising low viscosity nitrocellulose, an aliphatic alcohol selected from the group consisting of substantially anhydrous ethyl alcohol, isopropyl alcohol and tertiary butyl alcohol, and a supplementing fortifying solvent.

THEODORE F. BRADLEY.